

## UNITED STATES PATENT OFFICE

2,119,050

## LIQUID OXYGEN EXPLOSIVE

George Burkle Holderer, Scarsdale, N. Y.

No Drawing. Application August 19, 1937.  
Serial No. 159,914

## 6 Claims. (Cl. 52—1)

This invention relates to explosives and more particularly to liquid oxygen explosives.

In the use of liquid oxygen explosives a suitable amount of carbon or carbonaceous material is placed in a bag or wrapper or made into a cartridge, and liquid oxygen is added thereto. The cartridges actually used in this manner may be of considerable size and when they are to be used, they are placed or dropped in a hole or bore to be blasted, tamped in place and then detonated. The most serious objection to the use of liquid oxygen explosives has been that they are sensitive to sparks or flame. As a result, premature explosions have been caused by stones or other objects falling on the saturated cartridges as they are being lowered into drill holes or such explosions have been caused by shocks or sparks accidentally transmitted to the cartridges in transit. Many attempts have been made to overcome this fault. In the prior patent of George St. John Perrott and me, No. 1,860,816, granted May 31, 1932 we have disclosed and claimed a method of regulating the sensitivity of explosives of this type wherein an incombustible material in a finer state of division than the carbon is added to the carbon. Likewise in the Holderer and Clark Patent No. 1,865,104, granted June 28, 1932 we have disclosed and claimed the use of a binder in an amount sufficient to agglomerate the carbonaceous material without appreciably affecting its porosity, and in my prior Patent No. 1,960,907, granted May 29, 1934, I have disclosed and claimed the use of carbonized lignin residues having a moisture content greater than 8 percent.

While each of these methods has resulted in the production of liquid oxygen explosives which are safer to handle than would otherwise be the case, I have now found that the sensitivity of such cartridges to outside spark or flame influence can be greatly minimized by treating the carbonaceous material with a fire-proofing substance preferably in a solution. Likewise the bags or wrappers in which the carbonaceous material is contained may be impregnated with fire-proofing material. Any of the ordinary fire-proofing salts may be employed for this purpose. Of such salts I prefer to use either dibasic or monobasic ammonium phosphate. My invention, however, is not limited to the use of this particular salt and equivalents therefor calcium chloride, magnesium sulphate, sodium silicate, borax, sodium bromide, sodium tungstate, zinc chloride, tri-basic zinc phosphate, tri-basic magnesium phosphate, phosphoric acid, mono-

basic magnesium phosphate, boric acid, mono-basic zinc phosphate, aluminum sulphate, ammonium bromide, ammonium chloride and ammonium sulphate. Combinations of these or similar chemicals may be desirable both from the standpoint of effectiveness and cost and the invention includes the use of two or more of these materials together. Also wide latitude of the strength of solutions employed is within the scope of the invention and the strength employed is based largely on the cost of the chemicals as all degrees of combination are effective. A few examples follow:

|                              | Per cent |
|------------------------------|----------|
| Magnesium chloride           | 45 15    |
| Mono-ammonium-phosphate      | 55       |
| Borax                        | 60       |
| Ammonium-phosphate (mono)    | 40       |
| Ammonium-phosphate (dibasic) | 25       |
| Ammonium sulphate            | 75 20    |
| Zinc chloride                | 54       |
| Ammonium-phosphate (mono)    | 46       |
| Magnesium chloride           | 44       |
| Sodium phosphate (mono)      | 56 25    |

In practicing the invention the carbonaceous material is first treated with the fire-proofing material and then placed in the bags or casings in the usual way. I preferably employ a water soluble, fire-proofing material and as a specific example a solution of ammonium phosphate of desired strength may be first formed. The solution is then added to the carbonaceous material up to 20% by weight. The water and the fire-proofing material are allowed to remain in the carbonaceous material and the carbonaceous material then placed in bags and liquid oxygen added thereto in the usual manner.

Instead of using a water-soluble, fire-proofing material, a material that is not water-soluble may be employed and thoroughly mixed with the carbonaceous material before the liquid oxygen is added thereto.

The addition of the fire-proofing material in the amounts stated reduces the sensitivity of the completed cartridge to a point where it is safer to handle but not enough to destroy its usefulness. The cartridge so produced is thus capable of being detonated in the usual manner when desired but is less liable to premature explosions caused by stones or other objects falling on the cartridge as it is being lowered into drill holes and is also less liable to explosion by casual flames, such as cigarettes, sparks, etc.

The carbonaceous material, treated as above

described, may be employed in the usual wrappers or bags of cotton fabric or the bag or wrapper may also be treated with the fire-proofing agent. When the bag is to be treated, the solution is prepared as above described and containing about one gallon of water to one pound of the salt. The bags or the material from which the bags are to be made, are soaked in this solution and allowed to dry.

5 10 As an alternative procedure, the bag may be filled with a carbonaceous material in the usual way and then treated with the fire-proofing solution, either by spraying the finished bag or by coating it by placing it in a vessel or trough 15 containing the solution. In this way the bag will become saturated with the fire-proofing solution and an outer layer of the carbonaceous material near the bag will also become saturated. If such outer layer of the carbonaceous material is saturated, it is not necessary to saturate the carbonaceous material throughout as this treatment 20 is effective in stopping both flaming and glowing of the carbonaceous material.

While the present invention may be practiced 25 with any type of carbonaceous material capable of absorbing liquid oxygen, I prefer to employ granular carbons having a high degree of absorption for liquid oxygen or other explosives.

30 A granular carbon of the type commercially known as Bugbird carbon, made in accordance with the Bugbird Patents Nos. 1,706,871, 1,779,530 and 1,781,214, may be used. This material is obtained by carbonizing liquors rich in dissolved lignins, such as those derived from the manufacture of wood pulp by the alkali (soda) process. The carbonized lignin residues are leached to remove water soluble impurities and then submitted to a slight grinding action to reduce the grains to a more or less uniform size. This produces a granular carbon in which the largest grains are not more than about one-quarter inch 40 in their longest dimension and so that not more than about 25 percent of the material will pass through a 100 mesh screen.

45 I am aware of prior patents disclosing the

treatment of bags or casings of explosive cartridges with fire-proofing materials for the purpose of making them fire-damp-proof. Fire-damp-proofing is not to be confused with the treatment of the carbonaceous material itself for the purpose of decreasing the sensitivity of the cartridge. This phrase means reducing the flame temperature of the explosive mixture to reduce the possibility of igniting fire-damp, i. e., methane, carbon monoxide or coal dust, which is often present in mines. In such processes the treatment is confined to the cartridge casing to form a coating or crust on it and confine the flame when the explosion occurs. In the product of my invention the cartridge material itself is treated to lower its sensitivity to casual flame without affecting its ability to absorb liquid oxygen and without destroying its propulsive strength.

I claim:

- 20 1. A liquid oxygen explosive comprising carbonaceous material in granular form impregnated with a solution of a fire-proofing material.
2. A liquid oxygen explosive comprising carbonaceous material in granular form impregnated with a solution of ammonium phosphate.
- 25 3. A liquid oxygen explosive comprising carbonaceous material in granular form impregnated with a solution of calcium chloride.
4. The herein described method which comprises impregnating granular carbonaceous material with a solution of fire-proofing material, placing the material in a bag or casing and adding liquid oxygen thereto.
- 30 5. The herein described method which comprises impregnating granular carbonaceous material with a solution of ammonium phosphate, placing the material in a bag or casing and adding liquid oxygen thereto.
- 35 6. The herein described method which comprises impregnating granular carbonaceous material with a solution of calcium chloride, placing the material in a bag or casing and adding liquid oxygen thereto.

GEORGE BURKLE HOLDERER. 45